

# United States Patent Office

2,936,284

Patented May 10, 1960

1

2,936,284

## LUBRICATING OIL ADDITIVE COMPATIBILITY IMPROVER

Adlai E. Michaels, Cranford, and Niilo V. Hakala, Westfield, N.J., assignors to Esso Research and Engineering Company, a corporation of Delaware

No Drawing. Application October 24, 1955  
Serial No. 542,488

10 Claims. (Cl. 252—33.4)

This invention relates to methods of preparing improved lubricating oil compositions containing different additives having some degree of incompatibility. More particularly, it relates to methods of improving the compatibility of metallo-organic additives and polymeric additive materials in lubricating oil compositions. It relates also to lubricating compositions containing different additive materials exhibiting some degree of incompatibility to which have been added compounds which will be designated "compatibility improvers."

Lubricating oils manufactured by conventional methods are often unsuited for use under conditions encountered in internal combustion engines and for diverse industrial purposes. Satisfactory lubricating can be generally given by almost any type of lubricant of the proper viscosity for brief periods of time. However, for a sustained service under normal operating conditions the quality of lubricants becomes important and it is necessary for the lubricant not only to carry out the primary functions but also to exhibit the following advantages: (1) the lubricant should operate satisfactorily over a wide temperature range, and (2) the deleterious effects of excessive engine deposits should be countered. In order to achieve these performance objectives, important characteristics of lubricating oils must be enhanced, especially viscosity, viscosity index, pour point and ability to remove carbonaceous deposits. To obtain these and other desirable results, various additive materials have been blended with lubricating oils to extend the quality of lubricants for specific purposes beyond the level which can be reached by known manufacturing methods.

Generally, additives have been developed for specific purposes, for example, pour point depressants, viscosity index improvers, sludge dispersers, detergents, and the like. To obtain a general purpose lubricant having a high level of performance with respect to pour point, viscosity index, sludge dispersion, and the like, it is necessary to incorporate in the lubricating oil base stock many varied additive materials. Because of the diverse nature of many of these materials, it is not surprising that a certain incompatibility among them exists. For example, metallo-organic compounds used as detergent additives are frequently incompatible with high molecular weight polymeric materials used primarily as thickeners, viscosity index improvers, pour point depressors, etc. Lubricating oils having incorporated therein the above-mentioned additive materials are frequently unacceptable because of turbidity or because of viscosity instability, etc. It has also been found that certain of the metallo-organic additive materials actually reduce the effectiveness of certain of the polymeric addition agents. For instance it has been found that the pour point depressing potency of some of the additive materials is markedly reduced when blended with a metallo-organic sludge dispersing agent in an oil base.

It has now been discovered that the addition of certain oxygenated organic compounds of the glycol ether type improves the compatibility of metallo-organic addi-

2

tives and highly polymeric additives, and corrects thereby the unacceptable turbidity or viscosity increase of a lubricant using the two additives. It has also been found that the undesirable depreciation of pour point depressing potency is removed by the incorporation into the blend of these oxygenated organic compounds.

These oxygenated organic compounds may be represented by the formula:



where R is an alkyl group having 1 to 8 carbon atoms, R' is hydrogen or an alkyl group having 1 to 8 carbon atoms, and n is an integer from 1 to 8.

Among the operable oxygenated compounds covered by the formula above are the following:

|    |                                       |
|----|---------------------------------------|
| 20 | Ethylene glycol mono-methyl ether     |
|    | Ethylene glycol mono-ethyl ether      |
|    | Ethylene glycol mono-butyl ether      |
|    | Diethylene glycol mono-methyl ether   |
|    | Diethylene glycol mono-ethyl ether    |
|    | Diethylene glycol mono-butyl ether    |
|    | Triethylene glycol mono-methyl ether  |
|    | Triethylene glycol mono-ethyl ether   |
| 25 | Tetraethylene glycol di-methyl ether  |
|    | Polypropylene glycol monoalkyl ethers |
|    | Polypropylene glycol di-alkyl ethers  |

Oxygenated organic compounds of the class enumerated may be dissolved in oil mixtures or solutions which 30 contain incompatible additive materials for the purpose of minimizing or eliminating said incompatibility. These oxygenated compounds may be added (1) to the base oil before the addition of the polymeric additive or the metallo-organic additive, (2) to the oil blend after the 35 addition of either the polymeric additive or the metallo-organic additive, (3) to the oil blend after the addition of the polymeric additive and the metallo-organic additive, and (4) to the metallo-organic additive.

The oxygenated organic compounds are ordinarily 40 used in amounts varying between about 0.01% to 5.0% by weight, preferably 0.05% to 3.0% by weight.

The polymeric additive materials which have utility as viscosity index improvers and pour point depressants and which are found to be incompatible to some degree with the metallo-organic detergent inhibitors are the polymerized or copolymerized esters having ester chain lengths within a range of from 8 to 18 carbon atoms in a substantially straight chain. These additive materials are covered by the term "alpha,beta-unsaturated carboxylic acid ester polymers or copolymers." They include, among others, polymers and copolymers of esters of acrylic, methacrylic, crotonic and isocrotonic acid, esters of the dibasic acids, such as, maleic, fumaric, citraconic and mesaconic acid, copolymers of these acid esters with vinyl esters such as vinyl acetate, vinyl propionate, vinyl butyrate, vinyl caproate, vinyl laurate, and the like.

The preparation of these additive materials is accomplished by straight forward methods and present no problem to the art. Examples of the preparation of representative types are set out below:

### PREPARATION OF DI-ALKYL MALEATE ESTER

A 3-liter flask equipped with a water trap and a reflux condenser was washed with 294 g. of maleic anhydride, 1118 g. of the alcohol obtained by hydrogenation of coconut oil and containing an average of 13.5 carbon atoms per molecule, 2 g. of sulfosalicylic acid, 400 cc. of xylene, and 200 cc. of naphtha. The above mixture was refluxed for a total of 14 hours, during which time 58 cc. of water were collected. The reaction product was diluted with about 1,000 cc. of benzol and then given

four washes with 5% to 10% sodium carbonate solution and two with water. The solvents were removed by evaporation on a steam bath. The resulting maleate ester had a saponification number of 230, a neutralization number of 0.5, and a viscosity at 210° F. of 41.7 SUS and an average molecular weight of about 495.

#### COPOLYMERIZATION OF VINYL ACETATE WITH MALEATE ESTER

A 1-liter 3-necked flask equipped with a condenser, stirrer, and a thermometer was charged with 200 g. of a lubricating oil having a viscosity at 210° F. of 44 SUS and 300 g. of the maleate ester as prepared above. This mixture was heated to about 30° C. after which it was blown with nitrogen for about 5 minutes. There was then added 4 g. of benzoyl peroxide and the mixture was again blown with nitrogen for about 5 minutes. Vinyl acetate addition was started with stirring about 45 minutes after the addition of the benzoyl peroxide and a total of 100 g. of vinyl acetate was added during the course of 1½ hours. The reaction mixture was maintained at 80° C. with stirring for 20 hours from the first addition of the vinyl acetate. The resulting copolymer had a viscosity at 210° F. of 3042 SUS.

#### PREPARATION OF DI-ALKYL FUMARATE-VINYL ACETATE COPOLYMER

The di-alkyl fumarate ester of coconut alcohol was prepared by the direct esterification of fumaric acid with a mixture of alcohols obtained by hydrogenating coconut oil and having an average number of carbon atoms of about 13.5. The di-ester was then copolymerized with n-vinyl acetate in the presence of a small amount of benzyl heptane as a solvent and using a small amount of benzoyl peroxide as a catalyst. The exact amount of materials used are as follows:

650 g. coconut alcohol fumarate (1.31 mols)  
113 g. vinyl acetate (1.31 mols)  
85 cc. n-heptane  
7.63 g. 60-mesh benzoyl peroxide

The above charge was stirred for 17 hours 10 minutes at 70° C. under nitrogen atmosphere. n-Heptane and unreacted vinyl acetate were removed by evaporation at 80° C. under vacuum. The resulting copolymer product which was water-white and highly viscous had a molecular weight of about 7,100 Staudinger.

#### PREPARATION OF POLYMERIZED ACRYLATE AND METHACRYLATE ESTERS

The esters of acrylic and methacrylic acid are simply prepared by an ester interchange reaction using the desired alcohol, a C<sub>8</sub>-C<sub>18</sub> alcohol, and the methyl esters of the acids. Usually an acidic catalyst is used to promote the interchange. Polymers of the esters are prepared by heating the esters to a temperature for about 15 hours at about 100° C. in the presence of a small amount of benzoyl peroxide catalyst. Any unreacted ester may be removed by heating the product in a vacuum (0.5-1 mm. Hg) to a temperature just about the boiling point of the ester. The polymers obtained are usually colorless or faintly yellow.

The polymeric additive materials having viscosity index improving or pour point depressing properties are blended into lubricating oils in amounts between about 0.02% to 10% by weight, preferably 0.1% to 5.0%, percentages being by weight, based on the weight of the total composition.

The metallo-organic additive material having the desirable detergency-improving characteristics are preferably the metal salts of sulfonic acids, either natural or synthetic, metal salts of alkylated phenols, metal salts of sulfided alkyl phenol, or the reaction products of the metal salts of sulfided alkyl phenols and phosphorus sulfide. With these materials may be combined minor

amounts of other known additives, such as metal salts of compounds containing both sulfur and phosphorus, sulfurized hydrocarbons, and the like. The barium salt of the alkyl phenol sulfide is particularly useful either alone or reacted with phosphorus sulfide. Calcium sulfonate is an especially preferred sulfonate. These materials are well known in the art of their preparation and are described in detail in the literature. It has been found that oil compositions containing from 0.2% to 3.0% by weight of these detergent inhibitors, based on the weight of the total composition, have desirable detergent properties. A preferred range is from 0.8% to 2% by weight.

As is set out in detail above, the oil compositions of this invention comprise mineral lubricating oils containing combined therein (1) a copolymer material which imparts desirable properties of viscosity index improving and/or pour depression to the blend, (2) a metallo-organic additive which is useful for improving the detergency characteristic of the oil blend, and (3) a compatibility improver which serves to minimize or eliminate any turbidity or instability caused by a mixture of the metallo-organic additive and the copolymeric material.

In order to more explicitly define the invention outlined above, the following examples are given, it being understood that these examples are only illustrative of the inventive concept and not considered to be limiting in any way.

#### Example I

A solvent extracted Mid-Continent paraffinic oil having a Saybolt viscosity of 46 seconds at 210° F. and a viscosity index of 110 had added thereto 0.2% of an alkyl maleate-vinyl acetate copolymer prepared according to the technique outlined above. Ten separate samples of the above lubricating oil composition were set aside. To five of these samples were added 0.8% of five separate samples of inhibitor-detergents consisting of the barium salt of alkyl phenol sulfide reacted with phosphorus sulfide. All five blends were hazy or turbid initially and on several days standing, all blends were very turbid with a precipitate settling out in one blend. To the remaining five samples were added the same inhibitor-detergent additives but in this case the inhibitor-detergent additives contained diethylene glycol mono-ethyl ether (sufficient quantities to give a concentration of 0.02% in the final blend). After standing two and a half months, the latter samples were found to be perfectly clear.

#### Example II

Two samples were prepared as in Example I with the exception that a different alkyl dibasic acid ester-vinyl acetate copolymer was employed. The blend without the compatibility improver turned cloudy immediately, but the blend containing the diethylene glycol mono-ethyl ether (0.02% in final blend) was still clear at the end of the two and a half months examination period.

#### Example III

Two samples were prepared as in Example II except that in the one blend 0.04% diethylene glycol mono-ethyl ether was added directly to the oil blend before the addition of the detergent additive instead of as a component of the latter additive. The blend without the compatibility improver was cloudy immediately whereas the blend containing the diethylene glycol mono-ethyl ether was still clear at the end of two and a half months.

#### Example IV

Example III was repeated except that a different sample of alkyl dibasic acid ester-vinyl ester copolymer was employed and 0.02% instead of 0.04% compatibility improver was employed. Results were identical with those observed in Example III.

## Example V

Eight oil blends were prepared using the same test oil and the same polyester copolymer (0.2%) described in Example I. To four of the blends were added 2.0% of 4 separate samples of the detergent inhibitor employed in Example I plus calcium petroleum sulfonate. All four blends exhibited some haziness in one day. To the remaining four samples were added the same inhibitor-detergent additives but in this case the latter additives contained diethylene glycol mono-ethyl ether sufficient to give a final blend concentration of 0.025%. All of the

## Example IX

Two blends were prepared using the same base stock, same polyester copolymer and same detergent additive described in Example VIII. To one of the blends was added 0.04% dimethoxytetraethylene glycol. The blend without the compatibility improver was cloudy initially whereas the latter blend was clear initially but showed a slight haze at the end of a 40-day low temperature (40° F.) storage test.

10 The results of the above experiments may be summarized as follows:

TABLE I.—COMPATIBILITY OF POLYESTER COPOLYMERS WITH METALLO-ORGANIC ADDITIVES  
Blends contain 0.2% copolymer in extracted Mid-Continent oil having a Saybolt viscosity of 46 seconds at 210° F. and a viscosity index of 110.]

| Detergent Additive                                                                            | Appearance of Blend (Without Compatibility Improver) | Compatibility Improver                            | Appearance of Blend Containing Compatibility Improver |
|-----------------------------------------------------------------------------------------------|------------------------------------------------------|---------------------------------------------------|-------------------------------------------------------|
| 0.8% Metal salt of alkyl phenol sulfide+phosphorus sulfide.                                   | Turbid initially; precipitate on standing.           | 0.02% Diethylene glycol mono-ethyl ether.         | Clear end of 2½ months.                               |
| 0.8% Metal salt of alkyl phenol sulfide+phosphorus sulfide (4 samples).                       | Haze initially; very turbid in several days.         | do                                                | All clear end of 2½ months.                           |
| 1.0% Metal salt of alkyl phenol sulfide.                                                      | Light haze in one week.                              | 0.006% Diethylene glycol mono-ethyl ether.        | Do.                                                   |
| 0.8% Metal salt of alkyl phenol sulfide.                                                      | Slight haze in several days; cloudy—2 wks.           | do                                                | Clear end of 2½ months.                               |
| 2.0% Metal salt of alkyl phenol sulfide+phosphorus sulfide+calcium mahogany soap (4 samples). | Slight haze initially.                               | 0.025% Diethylene glycol mono-ethyl ether.        | All clear end of 2½ months.                           |
| 0.8% Metal salt of alkyl phenol sulfide+phosphorus sulfide.                                   | Turbid initially; very turbid on standing.           | 0.04% Methoxy triglycol <sup>1</sup>              | Clear end of 2½ months.                               |
| Do.                                                                                           | do                                                   | 0.02% Methoxy triglycol <sup>1</sup>              | Do.                                                   |
| Do.                                                                                           | do                                                   | 0.04% Dimethoxytetraethylene glycol. <sup>1</sup> | Clear initially. <sup>2</sup>                         |
| Do.                                                                                           | Cloudy initially.                                    | 0.02% Diethylene glycol mono-ethyl ether.         | Clear end of 2½ months.                               |
| Do.                                                                                           | do                                                   | 0.04% Diethylene glycol mono-ethyl ether.         | Do.                                                   |
| Do.                                                                                           | do                                                   | 0.02% Diethylene glycol mono-ethyl ether.         | Do.                                                   |

<sup>1</sup> Compatibility improver added directly to oil blend.

<sup>2</sup> Slight haze at end of 40-day low temperature (40° F.) storage test.

latter blends were clear after two and a half months standing.

## Example VI

Two oil blends were prepared using the same test oil and the same polyester copolymer (0.2%) described in Example I. To one blend was added 1.0% of a detergent-inhibitor comprising the metal salt of alkylated phenol sulfide and to the second blend was added 1.0% of the same additive containing diethylene glycol mono-ethyl ether (0.006% concentration in final blend). The first blend exhibited a slight haze in one week whereas the blend containing the compatibility improver was clear at the end of two and a half months.

## Example VII

Two oil blends were prepared using the same test oil and the same polyester copolymer (0.2%) described in Example I. To one blend was added 0.8% of calcium isooctyl phenol sulfide and to the second blend was added 0.8% of the same additive containing diethylene glycol mono-ethyl ether (0.006% concentration in final blend). The first blend exhibited a haze in several days and was cloudy in 2 weeks whereas the blend containing the compatibility improver was clear at the end of two and a half months.

## Example VIII

Three oil blends composed of 0.2% alkyl dibasic acid ester-vinyl acetate copolymer and the same base stock described in Example I were prepared. To one blend was added 0.8% of  $P_2S_5$  treated barium isooctyl phenol sulfide, to the second blend was added 0.04% methoxy triglycol and 0.8% of the same detergent additive and to the third blend was added 0.8% of the same detergent additive which contained methoxy triglycol (0.02% concentration in final blend). The first blend was cloudy immediately while the two blends containing the compatibility improver were clear at the end of two and a half months.

An examination of the data appearing in the table above points out the efficacy of the compatibility improver of this invention. In all instances, the initial turbidity was removed by the addition of minor amounts of the oxygenated compound as defined above.

The compatibility improvers of this invention also have the desirable feature of eliminating the depreciation of the pour point depressing potency which has been experienced when these polymeric additive materials are compounded in a base oil with the detergent-inhibitor additives. The desirable elimination of this loss in pour point depressing potency is illustrated by the following:

50

## Example X

Using as a lubricating oil base a highly refined Mid-Continent distillate of SAE 20 grade there was prepared a composition containing 0.02 wt. percent of a copolymer of 80% Lorol B fumarate and 20% vinyl acetate prepared as described above. The ASTM pour point of the blend was  $-25^{\circ}$  F. To enhance the detergent inhibiting properties of this blend there was added 5% by weight of a blend of calcium cetyl phenate which contained a small amount of sulfurized paraffin and a minor amount of zinc dialkyldithiophosphate. The pour point of the resulting composition was increased  $30^{\circ}$  to  $+5^{\circ}$  F. This composition was entirely unsuited for low temperature use. The second composition was prepared containing identical amounts of polymeric additive and the detergent-inhibitor and in addition 0.05% by weight of diethylene glycol mono-ethyl ether. The ASTM pour point of this blend was  $-25^{\circ}$  F. clearly showing the utility of the oxygenated organic compound.

70

## Example XI

To a highly refined Mid-Continent distillate of SAE 20 grade there was added 0.2 wt. percent of a polymerized methacrylate ester having an ester chain length of between 8 and 18 carbon atoms. The ASTM pour point of this blend was  $-30^{\circ}$  F. A blend containing the

same weight percent of the polymethacrylate ester in the same base stock and containing in addition 5 wt. percent of the detergent-inhibitor described in Example X above had an ASTM of  $-10^{\circ}$  F. A second blend containing identical amounts of the polymerized methacrylate ester and the detergent-inhibitor in the same base stock was prepared and in addition 0.05% by weight of a diethylene glycol mono-ethyl ether was added. The ASTM pour point of this final composition was  $-30^{\circ}$  F., pointing out that in this instance, like in Example X above, the depreciation of the pour point depressing potency of the polymerized methacrylate ester by the detergent inhibitor was removed.

*Example XII*

To show the viscosity stabilizing effect of the compatibility improvers on various blends containing both detergent inhibitors of the alkylated phenol-sulfide and petroleum sulfonate type and viscosity index improvers, twelve blends were made and submitted to storage stability tests. The blends were prepared by admixing the components, heating to about  $150^{\circ}$  F. for 15 minutes with stirring. Data are set out in the table below.

TABLE II

| Blend                                   | 1     | 2     | 3     | 4     | 5     | 6     | 7     | 8     | 9     | 10    | 11    | 12    |
|-----------------------------------------|-------|-------|-------|-------|-------|-------|-------|-------|-------|-------|-------|-------|
| Composition (Vol. Percent):             |       |       |       |       |       |       |       |       |       |       |       |       |
| Base Oil <sup>1</sup>                   | 94.7  | 92.7  | 96.2  | 94.2  | 95.2  | 93.2  | 94.7  | 90.7  | 92.7  | 93.7  | 94.95 | 95.2  |
| Polymethacrylate <sup>2</sup>           | 1.8   | 1.8   | 1.8   | 1.8   | 1.8   | 1.8   | 1.8   | 1.8   | 1.8   | 1.8   | 1.8   | 1.8   |
| Calcium Sulfonate                       | 1.2   | 1.2   | 2.0   | 2.0   | 2.0   | 2.0   | 1.2   | 1.2   | 1.2   | 1.2   | 1.2   | 1.2   |
| Ca-Ba Salt of Diisobutyl Phenol Sulfide | 1.1   | 1.1   |       |       |       |       | 1.1   | 1.1   | 1.1   | 1.1   | 1.1   | 1.1   |
| Zn Diallyl Dithiophosphate <sup>3</sup> | 0.6   | 0.6   |       |       | 0.6   | 0.6   | 0.6   | 0.6   | 0.6   | 0.6   | 0.6   | 0.6   |
| Phosphorus-treated Terpene              | 0.6   | 0.6   |       |       | 0.6   | 0.6   | 0.6   | 0.6   | 0.6   | 0.6   | 0.6   | 0.6   |
| Compatibility Improver <sup>4</sup>     |       | 2.0   |       |       | 2.0   | 2.0   |       | 4.0   | 2.0   | 1.0   | 0.75  | 0.5   |
| Test Results:                           |       |       |       |       |       |       |       |       |       |       |       |       |
| Viscosity (SUS/100° F.)—                |       |       |       |       |       |       |       |       |       |       |       |       |
| Of Original Blend                       | 218.8 | 222.2 | 308.0 | 300.7 | 339.9 | 308.3 | 324.9 | 301.3 | 312.7 | 309.7 | 321.9 | 326.0 |
| Viscosity Change After Storage of—      |       |       |       |       |       |       |       |       |       |       |       |       |
| 16 hrs.                                 | +1.8  | +0.2  | +2.8  | -0.4  | +4.8  | 0     | +4.4  | +0.3  | +0.5  | +0.2  | +1.1  | +1.3  |
| 40 hrs.                                 |       | -0.4  |       |       |       |       |       |       |       |       |       | -1.2  |
| 88 hrs.                                 | +4.5  |       | +6.1  | -0.7  |       | -0.2  | +5.2  |       |       |       |       |       |
| 168 hrs.                                |       |       |       |       |       |       | +7.4  | +0.3  | 0     | +0.2  |       |       |
| 456 hrs.                                | +6.4  |       |       |       |       |       |       |       |       |       |       |       |

<sup>1</sup> A solvent extracted Mid-Continent neutral, viscosity @  $210^{\circ}$  F. of 100 SUS in Ex. 1 and 2; in Ex. 3-12, an SAE 10W-30 base oil, Mid-Continent solvent extracted.

<sup>2</sup> A polymerized methacrylate ester containing Cr-10 in the ester groups. (Acryloid 763.)

<sup>3</sup> The alkyl groups correspond to the alkyl groups of methyl-isobutyl carbinol.

<sup>4</sup> Diethylene glycol mono-ethyl ether.

The data in the table above shows the effect of inclusion of the compatibility improvers of this invention in blends containing various additive materials. It is seen that the viscosity stability of the blends are greatly enhanced by the compatibility improver.

To summarize briefly, this invention relates to an oil composition which consists essentially of a mineral lubricating oil, from 0.5% to 10% of a polymerized alpha,beta-unsaturated carboxylic acid ester containing from 8 to 18 carbon atoms in the ester portion thereof and copolymers of such esters with vinyl esters, from 0.2 to 3.0% of a metallic salt of a petroleum sulfonic acid, a metal salt of an alkylated phenol, a metallic salt of a sulfided alkylated phenol, or the phosphorus sulfide reaction product of such metallic salts, and from 0.01 to 5.0% of a compatibility improver having the formula:



wherein R is an alkyl group containing from 1 to 8 carbon atoms, R' is hydrogen or an alkyl group containing from 1 to 8 carbon atoms, and n is an integer from 1 to 8.

The preferred embodiment contemplates the use of a copolymer of a dibasic acid ester containing from 10 to 16 carbon atoms in the ester portion thereof, with a vinyl ester, the barium salt of an alkylated phenol sulfide, and a diethylene glycol ether.

This is a continuation-in-part of application Serial No. 285,531, filed May 1, 1952, for the same inventors, and now abandoned, which in turn is a continuation-in-part of application Serial No. 214,652, filed March 8, 1951, now U.S. Patent 2,602,048.

What is claimed is:

1. A non-turbid lubricating oil blend which consists essentially of a mineral oil base stock having combined therein about 0.05% to about 10% by weight of a viscosity index improving material selected from the class consisting of polymerized alpha,beta-unsaturated carboxylic acid esters containing from about 8 to about 18 carbon atoms in the ester portion thereof and copolymers of such esters with vinyl esters, from about 0.2% to 3.0% by weight of a detergent inhibitor selected from the class consisting of metallic salts of sulfonic acids and from 0.01% to 5.0% of a material having the formula



15 wherein R is an alkyl group containing from 1 to 8 carbon atoms, R' is a radical selected from the group consisting of hydrogen and alkyl groups containing from 1 to 8 carbon atoms and n is an integer from 1 to 8.

2. A non-turbid lubricating oil blend which consists essentially of a mineral oil base stock having combined therein about 0.05% to about 10% by weight of a copolymer of a dibasic acid ester containing from 8 to 18 carbon atoms in the ester portion thereof and a vinyl

ester, from about 0.2% to 3.0% by weight of a detergent inhibitor selected from the class consisting of metal salts of sulfonic acids, and from about 0.05% to 3.0% by weight of a compatibility improver having the formula



50 wherein R is an alkyl group containing from 1 to 8 carbon atoms, R' is a radical selected from the group consisting of hydrogen and alkyl groups containing from 1 to 8 carbon atoms, and n is an integer from 1 to 8.

55 3. A non-turbid lubricating oil blend which consists essentially of a mineral oil base stock having combined therein about 0.1% to about 2.0% by weight of a copolymer of a fumarate ester containing from 8 to 18 carbon atoms in the ester portion thereof and a vinyl ester, from about 0.08% to 2.0% by weight of a detergent inhibitor selected from the class consisting of metal salts of sulfonic acids, and from about 0.05% to 4.0% by weight of a compatibility improver of the formula



60 65 wherein R is an alkyl group containing from 1 to 8 carbon atoms, R' is a radical selected from the group consisting of hydrogen and alkyl groups containing from 1 to 8 carbon atoms, and n is an integer from 1 to 8.

70 4. A lubricating oil blend according to claim 1 wherein said detergent inhibitor is calcium sulfonate.

5. A lubricating oil blend according to claim 1 wherein said compatibility improver is diethylene glycol mono-ethyl ether.

6. A lubricating oil blend according to claim 2 wherein 75 the detergent inhibitor is calcium sulfonate.

7. A lubricating oil blend according to claim 2 wherein said compatibility improver is methoxy triglycol.

8. A lubricating oil blend according to claim 2 wherein said compatibility improver is dimethoxy tetraethylene glycol.

9. A non-turbid lubricating oil blend which consists essentially of a mineral oil base stock having combined therein about 0.1% to about 2.0% by weight of a polymer of a methacrylate ester containing from 8 to 18 carbon atoms in the ester portion thereof, from about 0.8% to 2.0% by weight of a detergent inhibitor selected from the class consisting of metal salts of sulfonic acids, and from about 0.01% to 5.0% by weight of a compatibility improver having the formula



wherein R is an alkyl group containing from 1 to 8 carbon atoms, R' is a radical selected from the group consisting of hydrogen and alkyl groups containing from 1 to 8 carbon atoms, and n is an integer from 1 to 8.

10. A non-turbid lubricating oil blend which consists

essentially of a mineral oil base stock having combined therein about 0.1% to about 2.0% by weight of a copolymer of a maleate ester containing from 8 to 18 carbon atoms in the ester portion thereof and a vinyl ester, from about .08% to 2.0% by weight of a detergent inhibitor selected from the class consisting of metal salts of sulfonic acids, and from about 0.05% to 4.0% by weight of a compatibility improver of the formula



wherein R is an alkyl group containing from 1 to 8 carbon atoms, R' is a radical selected from the group consisting of hydrogen and alkyl groups containing from 1 to 8 carbon atoms, and n is an integer from 1 to 8.

References Cited in the file of this patent

UNITED STATES PATENTS

|           |                 |       |               |
|-----------|-----------------|-------|---------------|
| 2,383,915 | Morgan          | ----- | Aug. 28, 1945 |
| 2,602,048 | Michaels et al. | ----- | July 1, 1952  |
| 2,616,851 | Giammaria       | ----- | Nov. 4, 1952  |